

## UNITED STATES PATENT OFFICE.

HANS VON DAHMEN, OF VIENNA, AUSTRIA-HUNGARY, ASSIGNOR TO JOSEF FÜHRER, OF VIENNA, AUSTRIA-HUNGARY.

## DETONATING COMPOSITION.

SPECIFICATION forming part of Letters Patent No. 740,355, dated September 29, 1903.

Application filed November 21, 1903. Serial No. 132,844. (No specimen.)

*To all whom it may concern:*

Be it known that I, HANS VON DAHMEN, a subject of the Emperor of Austria-Hungary, residing at Vienna, in the Empire of Austria-Hungary, have invented new and useful Improvements in Detonating Compositions, of which the following is a specification.

For many years military authorities have been seeking a detonating composition which without the use of fulminates, picrates, or chlorates, or a nitro compound will fire explosives in a thoroughly-satisfactory manner, for at present the powerful explosives which are employed for filling shells render the use of the extremely-dangerous preparations of fulminic acid absolutely necessary as detonating agents.

The purpose of my invention is to overcome all the drawbacks at present experienced in the manufacture of explosives and to produce a detonating composition absolutely insensible to concussion, percussion, and friction. My new composition is more particularly adapted for artillery purposes.

In the manufacture of improved detonating compositions a mixture of potassium carbonate, sulfur, and potassium nitrate has been tried. The chemical change which here takes place is that the sulfur unites with the potassium carbonate to form potassium sulfite, which at a high temperature is suddenly oxidized by the potassium nitrate, nitrogen being liberated.

Potassium carbonate is of a highly-hygroscopic nature, so that a preparation of the above kind, apart from its deficient force, would be unsuitable for storing for any length of time. I therefore replace the carbonate by bicarbonate of potash, with the addition of aluminium.

By the admixture of aluminium the chemical decomposition of the compound mentioned is rendered much more energetic, the temperature being greatly increased.

In order to enable the above-mentioned explosives to be detonated in practice with the same success as with preparations of fulminate of mercury, my detonating composition must be employed in a particular manner. Its use in free space, it appears, is impracticable; but when confined in an air-

tight chamber it can be caused to exert a strong detonating effect. For this purpose the composition must be heated by a slow-buring ignition agent—such as ordinary black gunpowder or a mixture resembling such, Baumé's fusion-powder, (as described in Graham-Otto's *Ausführliches Lehrbuch der Chemie*, 5th edition, Vol. II, *Ausführliches Lehrbuch der Anorganischen Chemie*, 60 von Dr. A. Michaelis, Section III, page 147, lines 21-24) with or without the addition of aluminium, or by Goldschmidt's preparations, (such as are described in the *Chemisches Centralblatt*, 1898, II 84, 1899, II 459, Berlin.) In this manner the temperature of the composition is raised to that requisite for its thorough detonation.

For the purpose in view I take a detonating composition consisting, for instance, of nitrate of potash, 45.5 parts; bicarbonate of potash, thirty parts; sulfur, sixteen parts; aluminium, 8.5 parts. This I submit to pressure till the specific gravity is from one to two. Next I granulate it in well-known manner and then press from it plates or wafers some two millimeters thick. These are inserted as a bottom layer into the projectile-fuse in appropriate manner, depending upon the diameter of the latter. Upon such a plate I prefer to place a thin layer of tinfoil or other suitable medium, though such partition is not absolutely necessary. Hereupon I fill up the remaining space in the fuse with gunpowder or another of the heating agents of the kind already referred to, or instead of a plate, as stated above, I may employ the composition merely in granulated state, which in the case of pressed charges may also be filled into the fuse-hole or the projectile charge for the purpose of promoting more complete chemical decomposition, or the detonating composition may be employed in the form of powder or in pulverized or granulated form, mixed or pressed with the projectile charge, in which case naturally a heating agent, as above specified, must also be employed.

The admixture of about twelve per cent. of my detonating composition is sufficient to effect complete chemical decomposition of the ammonium preparations, which are well known to be extremely difficult to fire. This

simple manner of ignition can be readily adapted to any projectile, while insuring the highest degree of safety.

The detonating composition may be compounded in various ways, depending upon the kind of explosive employed. For example, the percentage of aluminium may be increased or diminished, accordingly as to whether a lower or higher temperature is required.

My new preparations, as already stated, are perfectly proof against concussion, percussion, and friction. By the sudden application of heat or by direct contact with fire they burn with a quiet flame without detonation. They keep for any length of time without decomposing. Thus by means of my new detonating composition I have attained what military authorities have long sought—viz., a safe priming composition for shells and projectiles which on the addition of a small quantity of powder or other slow-burning

composition possesses the same detonating effects as the dangerous fulminates, chlorates, or picrates hitherto in use. <sup>15</sup>

Having thus described my invention, what I claim as new, and desire to secure by Letters Patent, is—

1. A detonating composition consisting of potassium nitrate, bicarbonate of potash, sulfur and aluminium, substantially as described. <sup>20</sup>

2. A detonating composition consisting of potassium nitrate, bicarbonate of potash, sulfur and aluminium, to which is added a suitable slow-burning heating agent, substantially as set forth. <sup>35</sup>

In testimony that I claim the foregoing as my invention I have signed my name in presence of two subscribing witnesses.

HANS VON DAHMEN.

Witnesses:

HENRY HASPER,  
WOLDEMAR HAUPT.